

## UNITED STATES PATENT OFFICE

2,673,812

## METHOD OF PRODUCING CARBONACEOUS MOLDING COMPOSITIONS

Charles Desmond Greaves and Bernard Roy Atkins, London, England, assignors to C. D. Patents Limited, London, England, a British company

No Drawing. Application August 25, 1950,  
Serial No. 181,586

Claims priority, application Great Britain  
August 30, 1949

2 Claims. (Cl. 106—193)

1

This invention relates to improvements in the manufacture of carbonaceous moulding compositions and more particularly, but not exclusively, to the manufacture of such composition as are suitable for extrusion moulding in which a high degree of softness or plasticity is desirable.

There have previously been proposed in United States Patent specifications Nos. 2,461,365 and 2,493,383 methods of making moulded products from finely-divided bituminous coal without a binding agent in which an intimate mixture of finely-divided coal having good agglutinating properties with a swell-inhibiting agent is moulded and subsequently fired at a controlled rate of increase in temperature to a temperature above 550° C. under non-oxidising conditions, the method being so carried out that the resulting moulded product is not swollen, has a density greater than that of the coal used and has no cellular structure visible to the naked eye.

The use of such methods of dry powder moulding places limitations upon the shape of the articles that can be produced.

Again there has been proposed in specification of United States Patent application Serial No. 53,992 now Patent 2,640,787 and in specification of United States Patent application Serial No. 95,890 now Patent 2,637,072 a method of making from coal a carbonaceous moulding composition, especially an extrusible composition, which method consists in mixing at an elevated temperature subdivided coal and a softening agent which exercises a solvent action upon the coal and consists of hydrocarbon material such as coal tar oil, anthracene oil and the like. Such a mixture may be moulded to the desired shape at a temperature at which the mixture will flow and the moulded shape is fired under non-oxidising conditions at a controlled rate of temperature rise. Such processes may in certain cases be inconvenient because (1) the softening agent may exercise an action upon the coal, the properties of which are in consequence modified, (2) the swelling tendency may be increased, and (3) the softening agent may be unpleasant to handle or may produce fumes during the firing operation.

The main object of the present invention is to provide a method of producing a carbonaceous moulding composition in which no substantial modification of the original coal is produced.

The present invention consists in a method of producing a carbonaceous moulding composition which method comprises an intimate mixing of subdivided coal, water and a special lubricat-

2

ing agent comprising one or more carboxyl-substituted celluloses such for example as carboxy-methyl cellulose. Sodium carboxy-methyl cellulose has proved very successful.

This invention also includes a method of producing a moulded carbon product, which method comprises the submission of the carbonaceous moulding composition above referred to to a moulding or shaping operation and the subsequent heating of the shaped article under non-oxidising conditions and at a rate of temperature rise controlled so as to prevent intumescence, to a temperature of over 550° C.

The consistency of the moulding composition of the invention is governed by the quantity of water present which will not in general exceed 25–30 per cent, this percentage being dependent on the degree of subdivision of the coal. Hence during mixing care must be taken to limit loss of water by evaporation.

It may sometimes be desirable to add to the moulding composition a small proportion of a wetting agent. Suitable wetting agents are soaps, sulphated or sulphonated hydrocarbon derivatives or members of the "non-ionogenic" class of detergents. The mount of wetting agent employed varies with the circumstances but would generally be less than three per cent by weight of the mixture and must on no account be sufficient to exercise an oxidising or other chemical action upon the coal.

The amount of the special lubricating agent employed is so small that the amount of oxygen contained therein (in the cellulosic and carboxyl groups) is not sufficient to have a deleterious effect on the coal and the effect of such oxygen is to some extent balanced by the hydrogen present in the alkyl groups.

Sulphur, selenium or other substances having similar dehydrogenating properties may be added to the mixture, but care must be taken to select only such substances as are non-reactive to water, and they are preferably either finely-divided solids, or liquids which are readily miscible with water or which are dispersed in a medium containing not more than 30 per cent of water. The proportion of sulphur for example may be about 2% by weight of the coal. By the term non-reactive to water is meant that the substances used shall not react to any substantial degree with water under the conditions existing during the course of the process of preparing the moulding composition. Other finely-divided substances may be added which exercise the function of further reducing the swelling tendency of the coal or which confer special proper-

ties on the final product. Examples of such substances are carbon black, finely-divided graphite and china clay.

The coals most suitable for use in producing the composition of the invention are those having from 13 to 30 per cent of volatile matter calculated on the dry ash-free basis, but preferably coals having a volatile matter content of between 14 and 25 percent are employed.

The particle size of the subdivided coal may be such that 90 per cent passes through a 100-mesh sieve but is conveniently such that the average particle size lies between 6 and 30 microns.

The mixing of the coal, water and wetting agent may be suitably carried out at a temperature of 35° C. but higher or lower temperatures may be satisfactorily employed. The mixing operation may advantageously be effected over a period of 2 to 3 hours.

The moulding compositions of the invention may if desired be de-aerated, e. g. in a de-aerating mill before submitting to extrusion moulding which may either be effected at normal room temperature or at an elevated temperature, for example, 50° C.

After shaping or moulding the composition by extrusion or otherwise the moulded article is dried either in the air or by any other convenient and well known means, care being exercised that the drying is uniform so that the article remains free from cracks or distortion. It is found that, whereas immediately after extrusion the rods, tubes etc. produced thereby may require considerable care in handling, after drying they are easily handled.

#### Example I

700 lbs. of a mixture consisting of 70% of a South Wales strongly coking coal and 30% of graphite were ground together in a colloidal mill to a state of fine subdivision. The above mixture was placed in a Z-blade type of mixer and to this was added 268 lbs. of a jelly containing 94% of water, 5% sodium methylcarboxy cellulose and 1% of a wetting agent sold under the registered trade mark (Lissapol N); these additives having been previously mixed to a smooth consistency. (Lissapol N has the formula:



where R is a benzenoid ring and n is a whole number of 8 or more.) Mixing then took place for a period of 2 hours during which the temperature rose to 35° C. and the mixture developed a plastic consistency. The resulting mixture was then formed into a cylindrical billet by tamping in order to expel extrapped air and the billet so produced was extruded in the form of a tube. These tubes were then placed in an oven, maintained at 50° C. for 24 hours, after which they

were packed in powdered coke in boxes which were then placed in an electric furnace, the temperature of which was then raised to 850° C. at the rate of 2° C. per minute; the tubes were removed from the furnace after having been allowed to cool to approximately 200° C. under non-oxidising conditions.

#### Example II

4076 grammes of a mixture consisting of 70% South Wales strongly coking coal and 30% of graphite together with 75 grammes of sodium carboxymethyl cellulose were placed in a mixer of the edge-runner type and to this was added a solution of 15 ccs. of a wetting agent sold under the registered trade mark (Lissapol N) dissolved in 1410 grammes of water. The whole was then mixed for 2 hours during which the temperature rose to 25° C. and the mixture was then extruded and fired as in Example I.

We claim:

1. A method of producing a carbonaceous moulding composition which comprises the steps of intimately mixing finely sub-divided coal, water, between 1% and 2.5% by weight of the coal of sodium carboxymethyl cellulose, and a dehydrogenating agent non-reactive to water selected from the group consisting of sulfur and selenium, said agent comprising about 2% by weight of the coal.
2. A method of producing a carbonaceous moulding composition which comprises the steps of intimately mixing over a period of two to three hours sub-divided coal of average particle size between 6 and 30 microns, water, between 1% and 2.5% by weight of the coal of sodium carboxymethyl cellulose, less than 3% by weight of the mixture of a water-soluble wetting agent, the water constituting between 25% and 30% of the weight of the mixture, and the temperature during mixing being regulated to avoid appreciable water loss by evaporation.

CHARLES DESMOND GREAVES.  
BERNARD ROY ATKINS.

#### References Cited in the file of this patent UNITED STATES PATENTS

| Number    | Name    | Date         |
|-----------|---------|--------------|
| 2,461,365 | Bennett | Feb. 8, 1949 |
| 2,552,597 | Smith   | May 15, 1951 |

#### FOREIGN PATENTS

| Number  | Country       | Date         |
|---------|---------------|--------------|
| 2,577   | Great Britain | 1867         |
| 329,437 | Great Britain | May 22, 1930 |

#### OTHER REFERENCES

Hercules, "CMC" Hercules Pwd. Co., Wilmington, Del., 1946, p. 4.